

# United States Patent Office

3,280,030

Patented Oct. 18, 1966

1

3,280,030

## LUBRICATING COMPOSITION

Edward L. Kay, Akron, Ohio, and Edwin C. Knowles and William R. Siegart, Poughkeepsie, and Frederic C. McCoy, Beacon, N.Y., assignors to Texaco Inc., New York, N.Y., a corporation of Delaware  
No Drawing. Filed Sept. 10, 1963, Ser. No. 307,782  
7 Claims. (Cl. 252—49.7)

The present invention relates to a lubricating composition and, in particular, to mineral oil and synthetic ester base lubricating oils containing a complex or adduct of an inorganic halide and an amine to improve the load carrying properties of the lubricating composition.

New designs and improvements in machinery are continually raising the operating performance standards of lubricating compositions. In many instances, the pressures and temperatures to which the bearing surfaces of machinery operate under are higher than those which natural or synthetic lubricating oils can withstand. Instances where difficult lubricating conditions are encountered occur in the lubrication of heavily loaded pinion and spur gears, gear trains, bearings, extrusion applications and the like. As a result, there is an increasing need for lubricating compositions having improved properties for these services.

A class of lubricating compositions has been discovered which possesses greatly improved properties for a variety of lubricating applications. These compositions are particularly notable for their improvement in load carrying properties but many of them also possess additional valuable features, such as corrosion resistance, oxidation resistance and stability. These compositions provide the answer to some heretofore difficult lubricating problems.

The present lubricating composition comprises a major proportion of a lubricating oil base, such as a mineral lubricating oil or a synthetic lubricating oil, and a minor amount of an oil-soluble adduct formed between a hydrocarbylamine and an inorganic halide. More particularly, the additive of this invention is represented by the following formula:



wherein R is a hydrocarbyl radical having from 6 to 30 carbon atoms, R' and R'' are hydrogen or a hydrocarbyl radical having from 1 to 30 carbon atoms, the sum of the carbon atoms in R, R' and R'' being at least 12, y is an integer from 1 to 6, M is a polyvalent cation selected from the class consisting of aluminum, titanium, tin, zinc, copper, cadmium, magnesium, mercury, zirconium, antimony, bismuth, manganese, and iron, X is a halogen selected from the group consisting of chloride, bromide and iodide ions and in the case of divalent tin and the cations having a valence of 3 to 4 the fluoride ion, and z is an integer from 2 to 4 equal to the valence of M.

The adducts of the invention are prepared by mixing one to six moles of a hydrocarbylamine defined above with a mole of the halide compound from the class set forth. Simple mixing of the reactants will generally produce the reaction. Optionally, the reaction can be effected in the presence of a solvent. Solvents which are suitable are those which can dissolve the inorganic compound. Particularly effective solvents include acetone, methanol and tetrahydrofuran. This reaction is usually exothermic and provision must generally be made for cooling the reaction mixture. Caution must be exercised to keep the reaction temperature below the decomposition temperature of both of the components of the reaction product which generally means conducting the reaction at a tem-

2

perature below about 200° C. The reaction generally goes to completion in a short reaction time.

Amines which can be employed for preparing the adduct of the invention are those amines having one or more hydrocarbyl radicals and in which the total number of carbon atoms in said radicals is at least 12. The requirement of 12 carbon atoms in the amine is critical to insure the oil solubility of the adduct. Adducts having less than 12 carbon atoms are generally not soluble in lubricating oils. The effective amines including primary, secondary and tertiary amines correspond to the formula:



wherein R is a hydrocarbyl radical having from 6 to 30 carbon atoms. R is generally a branched chain alkyl radical because of the ready availability of these materials. Preferably, R is a tertiary alkyl radical having from 12 to 30 carbon atoms. R may, however, be an aryl, aralkyl or alkaryl radical having the prescribed number of carbon atoms. R' and R'' each represent hydrogen or a hydrocarbyl radical having from 1 to 30 carbon atoms of the same types defined for R. The sum of the carbon atoms in R, R' and R'' as noted above is at least 12.

Examples of the effective amines include laurylamine, tricaprylamine, di - 2 - ethylhexylamine, tridecylamine, tetradecylamine, hexadecylamine, octadecylamine, eicosylamine, tricosylamine, noncosylamine, nonylphenylamine, dodecylphenylamine, methyl dodecylamine, dimethyl dodecylamine, methyl octadecylamine and dimethyl octadecylamine. Particularly preferred amines are certain commercially available mixtures of tertiary alkyl primary amines. For example, a mixture of tertiary alkyl primary amines in which the alkyl radical comprises a mixture of alkyl groups having 11 to 14 carbon atoms is available under the name Primene 81-R. Another commercially available amine is the mixture of tertiary alkyl primary amines in which the alkyl radical comprises a mixture of alkyl groups having 18 to 24 carbon atoms 40 is available under the name of Primene JM-T.

Halides of metals and metalloids which can be employed to form the load carrying adducts of the invention include aluminum trichloride, aluminum trifluoride, titanium tetrachloride, titanium tetrafluoride, stannous chloride, stannous fluoride, stannic chloride, cupric chloride, 45 cupric bromide, cadmium chloride, cadmium iodide, magnesium chloride, mercuric chloride, zirconium chloride, antimony chloride, antimony fluoride, bismuth chloride, manganese chloride, ferric chloride, zinc chloride, zinc bromide and zinc iodide. The preferred halides are those formed from titanium, tin, aluminum, antimony, zinc and copper.

Only specific halides as set forth above are effective for producing the adducts of the invention. Examples of 55 halides which do not form adducts include cuprous chloride, cupric fluoride, magnesium fluoride, manganous fluoride, antimony oxychloride, barium chloride, lithium chloride and calcium chloride.

An unexpected phenomenon is the discovery that the 60 inorganic salt must have a substantial and apparently a critical degree of water solubility in order to form a complex with an amine of the type disclosed herein. The reason for the relationship between water solubility and complex formation is not fully understood. It has been determined, however, that the following critical conditions 65 must be met in order to form a complex of the type disclosed:

(A) The metallic element of the salt must be capable of sharing the unpaired electron of the amine nitrogen.

(B) The salts must have a water solubility greater than 70 0.2 mole per liter at a temperature in the range of 15-100° C.

Examples of inorganic salts and their behavior toward complex formation with a  $C_{21}$  primary amine (Primene JM-T) is given in Table I below:

TABLE I

| Salt      | $H_2O$ Solubility, Mols Salt/l. of $H_2O$ | Complex Formation With $C_{21}$ Primary Amine |
|-----------|-------------------------------------------|-----------------------------------------------|
| Zn $Cl_2$ | 45.3 (100° C.)                            | Yes.                                          |
| Zn $F_2$  | 0.15 (95° C.)                             | No.                                           |
| Sn $Cl_2$ | 14.2 (15° C.)                             | Yes.                                          |
| Sn $F_2$  | 2.68 (18° C.)                             | Yes.                                          |
| Zn $Br_2$ | 30.0 (100° C.)                            | Yes.                                          |
| Hg $Cl_2$ | 2.2 (100° C.)                             | Yes.                                          |
| Hg $Cl_2$ | 0.00002 (43° C.)                          | No.                                           |

The hydrocarbylamine and halide are reacted in the proportion of one to six moles of hydrocarbylamine to one mole of the halide compound with the preferred amount of the hydrocarbylamine being from one to four moles. Examples of adducts of the invention and the mole ratios of the components from which they were formed include the following:

Primene JM-T:aluminum trichloride (3:1),  
 Primene JM-T:tin tetrachloride (4:1),  
 Primene 81-R:aluminum trichloride (1:1),  
 Primene 81-R:titanium tetrachloride (2:1),  
 Primene 81-R:titanium tetrachloride (4:1),  
 Primene JM-T:titanium tetrachloride (4:1),  
 Primene JM-T:mercuric chloride (2:1),  
 Primene JM-T:ferric chloride (2:1),  
 Primene JM-T:cupric chloride (2:1),  
 Primene JM-T:antimony fluoride (3:1),  
 Primene JM-T:cadmium chloride (2:1),  
 Primene JM-T:cadmium iodide (2:1),  
 Primene JM-T:magnesium chloride (2:1),  
 Primene JM-T:zirconium chloride (2:1),  
 Primene JM-T:bismuth chloride (2:1),  
 Primene JM-T:antimony chloride (2:1),  
 Primene JM-T:zinc chloride (2:1),  
 Primene JM-T:zinc bromide (2:1), and  
 Primene JM-T:zinc iodide (2:1).

Examples of other suitable adducts include:

Primene 81-R:stannic chloride (2:1),  
 Tricaprylylamine:aluminum chloride (2:1),  
 Tricaprylylamine:titanium tetrachloride (2:1),  
 Di-2-ethylhexylamine:stannic chloride (2:1),  
 Di-2-ethylhexylamine:titanium tetrachloride (2:1), and  
 Di-2-ethylhexylamine:stannous fluoride (2:1).

The lubricating compositions of the invention are prepared by blending in a conventional way a minor amount of the oil-soluble, load-carrying hydrocarbylamine-halide adduct described hereinabove into a suitable lubricating oil base. Generally, the adduct is employed in an amount in the range of 0.05 to 10 percent by weight based on the weight of the lubricating composition with the preferred proportions being from 0.1 to 3 weight percent.

The base lubricating oil can be a mineral lubricating oil or a synthetic lubricating oil. The mineral lubricating oil can be a predominantly paraffinic or naphthenic or it can be a mixture of both types of mineral oils. Generally, the mineral oil will be a refined oil of predominantly paraffinic nature having a viscosity in the range from 30 to 150 Saybolt Universal Seconds at 210° F.

Various types of synthetic lubricating oil bases can be employed in preparing the lubricants of the invention. Aliphatic ester, polyalkylene oxides, silicones, esters of phosphoric and salicyclic acid and the highly fluorine-substituted hydrocarbons can be employed. Examples of the aliphatic esters include di-(2-ethylhexyl) sebacate, the dialkyl azelates, dialkyl suberates, and the dialkyl adipates such as di-hexyl azelate, di-(2-ethylhexyl) azelate, di-3,5,5-trimethylhexyl glutarate, di-(2-ethylhexyl) adipate, tri-amyl tricarballylate, etc. The polyalkylene oxides in-

clude polypropylene oxide, polyisopropylene oxide diether, polyisopropylene oxide diesters, etc. The silicones include methyl silicone, methylphenyl silicone, and the silicates include tetraisoctyl silicate. The highly fluorinated hydrocarbons include fluorinated oil, perfluorohydrocarbons, etc.

Other effective synthetic lubricating oils include the neopentyl glycol esters such as the neopentyl glycol propionates, neopentyl glycol butyrates and neopentyl glycol caprylates and the trimethylol alkanes such as trimethylol ethane, trimethylol propene, trimethylol pentane, trimethylol heptane and trimethylol dodecane and the like. Examples of the phosphate esters include tricresyl phosphate, trioctyl phosphate and tridecyl phosphate as well as mixed aryl and alkyl phosphates.

The load carrying ability of the lubricating compositions of the invention was determined by preparing mixtures of a mineral lubricating oil and a minor amount of a hydrocarbylamine-halide adduct of the invention and testing these lubricating compositions in the IAE Gear Test as a criterion of the load carrying activity. The IAE Gear Test, which is described in British specification DERD 2487, is carried out in gears having a non-indexed type motion under a load of at least 40 pounds. The load carrying gears in this test were operated at a speed of 6,000 r.p.m. The effectiveness of the lubricants of the invention is shown in the Table II below:

TABLE II  
IAE gear test, 6,000 r.p.m.

|    | Weight percent of adduct in Lubricating Comp.                                                                                                                                                                    | Tooth Load, Lbs. |
|----|------------------------------------------------------------------------------------------------------------------------------------------------------------------------------------------------------------------|------------------|
| 35 |                                                                                                                                                                                                                  |                  |
| 40 | Mineral Oil a Lubricating Compositions—Mineral Oil a plus adduct (adduct mole ratio):<br>1. Primene JMT. $AlCl_3$ (3:1) 2.1 73<br>2. Primene JMT. $TiCl_4$ (4:1) 2.0 77<br>3. Primene JMT. $SnCl_4$ (4:1) 0.6 88 | 18               |

a The mineral oil employed was a solvent refined paraffin base distillate having an SUS viscosity at 100° F. of about 130.

It is evident that the adduct-containing lubricating compositions were improved in their load carrying properties in the order of four to eight fold in comparison to the load carrying properties of the straight mineral oil.

The anti-scuffing and load carrying ability of a number of the lubricating compositions was determined in the well known Ryder Gear Test (Federal Test Method 6508). In this test, the lubricant is employed to lubricate two spur gears in a Pratt and Whitney Gear and Lubricating Tester (also called the Ryder Gear Tester). This tester was operated with a gear speed of 10,000 r.p.m. and with an oil inlet temperature of 165° F. A loading pressure of 5.0 p.s.i. was applied during break-in. After ten minutes, the tester was shut down and the gear examined for the percentage of tooth area scuff on each tooth. The procedure was then repeated using high load pressures with increments of 5 p.s.i. until 22.5 percent of the total tooth face area on the driving gear had been scuffed, the load applied in this run being considered the scuff load. The tooth load in pounds per inch of tooth width was then calculated.

The load carrying properties of some of the lubricating compositions was also determined by the Mean Hertz Load Test. This test is run in a machine having four  $\frac{1}{2}$ -inch diameter bearing balls which are driven under load while the balls are lubricated by the composition under test. This test is described in U.S. 2,600,058.

The lubricating compositions employed were prepared from two different base oils. Base Oil A was a mineral lubricating oil having an SUS viscosity at 210° F. of about 100. Base Oil B was a mineral lubricating oil hav-

ing an SUS viscosity at 210° F. of about 54. All the lubricant compositions contained 1 percent by weight of the indicated hydrocarbylamine-metal halide adduct. The results of this test are given in Table III below.

TABLE III

*Anti-scuff, anti-wear properties in Ryder Gear and Mean Hertz Load Tests*

| Nature of Adduct                       | Mole Ratio | Base Oil | Ryder Gear Test, p.p.i. | Mean Hertz Load |
|----------------------------------------|------------|----------|-------------------------|-----------------|
| Primene JMT/AlF <sub>3</sub>           | 2:1        | Oil A    | 2,660                   | 27              |
| Primene JMT/SnF <sub>2</sub>           | 2:1        | do       | 3,815                   | -----           |
| Primene JMT/TiF <sub>4</sub>           | 2:1        | do       | 4,000                   | -----           |
| Primene JMT/SbF <sub>3</sub>           | 3:1        | do       | 4,330+                  | 56              |
| Primene JMT/CuCl <sub>2</sub>          | 2:1        | Oil B    | 18                      | -----           |
| Primene JMT/HgCl <sub>2</sub>          | 2:1        | do       | 28                      | -----           |
| Tricaprylylamine/ZnCl <sub>2</sub>     | 2:1        | do       | 35                      | -----           |
| Di-2-ethylhexylamine/ZnCl <sub>2</sub> | 2:1        | Oil A    | 36                      | -----           |
|                                        |            | do       | 43                      | 20              |

The test results show that the lubricating compositions of the invention have substantially improved anti-scuff, anti-wear properties. The load carrying properties exhibited are particularly valuable in lubricants for gas turbines.

In the following tests, the extreme pressure and wear properties and anti-scuff properties were determined in lubricating compositions in which a synthetic base oil was employed. Base Oil C consisted of di-2-ethylhexyl sebacate plus sebacic acid which is commercially available as Plexol-2011. The properties of these lubricating compositions were determined in the Mean Hertz Load Test and the Navy Four Ball Wear Test.

The Navy Four Ball Test is a test for determining the anti-wear properties of a lubricant. The test machine comprises a system of 4 steel balls, 3 of which are in contact with each other in one plane in a fixed, triangular position in a reservoir containing the oil sample and a fourth ball above and in contact with the other three. In carrying out the test, the upper ball is rotated while it is pressed against the lower three at any desired pressure by means of a suitable weight applied to a lever arm, and the diameters of the scars on the three lower balls are measured by the means of a low power microscope. The average diameter, measured in two directions on each of the three lower balls, is taken as a measure of the anti-wear characteristics of the lubricant. The results of these tests are given in Table IV below.

TABLE IV

*Effect of concentration on EP, wear and anti-scuff properties of complexes*

| Oil Composition (wt.)                            | MHL | Navy Four Ball Wear, micron/min. |
|--------------------------------------------------|-----|----------------------------------|
| Base Oil C                                       | 16  | 11.8                             |
| Base Oil C plus 1% Primene JM-T/SbF <sub>3</sub> | 56  | 3.9                              |
| Base Oil C plus 2% Primene JM-T/SbF <sub>3</sub> | 50  | 5.3                              |
| Base Oil C plus 3% Primene JM-T/SbF <sub>3</sub> | 59  | 3.9                              |

The lubricating compositions containing the above-described hydrocarbylamine-metal halide adducts have

substantially improved extreme pressure, anti-wear and anti-scuff properties. They also exhibit good corrosion resistance, oxidation resistance and storage stability. These valuable properties make the lubricants of the invention suitable for a broad range of lubricating applications.

It is understood that the lubricating compositions of the invention can contain numerous additives conventionally used to improve the properties of lubricating oils. Commonly employed additives are the methacrylates as V. I. improvers and pour point depressors, the alkylphenols as oxidation inhibitors, alkaline earth metal salts of petroleum sulfonates or alkaryl sulfonates as detergents, metal di-alkyl dithiophosphate corrosion inhibitors and silicone anti-foam fluids.

Obviously, many modifications and variations of the invention as hereinbefore set forth may be made without departing from the spirit and scope thereof and, therefore, only such limitations should be imposed as are indicated in the appended claims.

We claim:

1. A lubricating composition comprising a major proportion of a lubricating oil and 0.05 to 10 percent by weight of an oil-soluble adduct of a hydrocarbylamine and titanium tetrafluoride having the formula:



wherein R is a hydrocarbyl radical having from 6 to 30 carbon atoms, R' and R'' are selected from the group consisting of hydrogen and a hydrocarbyl radical having from 1 to 30 carbon atoms, the sum of the carbon atoms in R, R' and R'' being at least 12, and y is an integer from 1 to 6.

2. A lubricating composition according to claim 1 in which said hydrocarbylamine is a C<sub>12</sub>-C<sub>30</sub> primary alkylamine.

3. A lubricating composition according to claim 1 containing 0.1 to 3 weight percent of said adduct.

4. A lubricating composition according to claim 1 in which said lubricating oil is a mineral lubricating oil.

5. A lubricating composition according to claim 1 in which said lubricating oil is a synthetic lubricating oil.

6. A lubricating composition according to claim 1 in which said lubricating oil is a dicarboxylic acid ester base oil.

7. A lubricating composition according to claim 1 in which said adduct consists of C<sub>18-24</sub> alkyl primary amine:titanium tetrafluoride in the mole ratio of 2:1 respectively.

#### References Cited by the Examiner

#### UNITED STATES PATENTS

|           |         |            |            |
|-----------|---------|------------|------------|
| 2,181,915 | 12/1939 | Rosen      | 252-49.6 X |
| 2,278,851 | 4/1942  | Hillman    | 252-49.7 X |
| 2,611,746 | 9/1952  | Kipp       | 252-49.6   |
| 3,076,835 | 2/1963  | Kay et al. | 252-49.6 X |

#### FOREIGN PATENTS

|    |         |        |                |
|----|---------|--------|----------------|
| 60 | 505,433 | 8/1954 | Canada.        |
|    | 833,397 | 4/1960 | Great Britain. |

DANIEL E. WYMAN, Primary Examiner.

P. P. GARVIN, W. H. CANNON, Assistant Examiners.